

Nov. 12, 1935.

O. C. ROHDE

2,020,967

SPARK PLUG AND METHOD OF MAKING THE SAME

Filed Sept. 21, 1934

FIG. 1.



FIG. 2.



FIG. 3.



Inventor

Otto C. Rohde

By *Owen & Owen*

Attorneys

## UNITED STATES PATENT OFFICE

2,020,967

SPARK PLUG AND METHOD OF MAKING  
THE SAME

Otto C. Rohde, Toledo, Ohio, assignor to Champion Spark Plug Company, Toledo, Ohio, a corporation of Delaware

Application September 21, 1934, Serial No. 744,949

9 Claims. (Cl. 29—84)

This application relates to a spark plug and method of making the same. More particularly it relates to a novel method of securing an electrode in a spark plug core and the core in the shell, and the structure resulting from this method.

Considerable difficulty has been encountered in satisfactorily sealing the central electrode in the usual spark plug core of porcelain or the like, and in permanently securing the core in its metallic shell. These difficulties arise from the differences between the materials of which the several parts are made and their action under the trying heat variations to which a spark plug is subjected in use.

In my co-pending application for Spark plug and method of making the same, filed February 9, 1934, Serial No. 710,459, I have disclosed and claimed an improvement whereby the electrode is sealed in the core by compacting soapstone or the like around the electrode in the core of the bore. By my present improvement I have simplified and somewhat improved the sealing of the electrode in the core, and likewise have provided for a similar sealing of the core in its shell. This improvement comprises as an important element the use of a compacting powder having a relatively low angle of repose, as will be pointed out more fully as the description proceeds.

In the accompanying drawing, Figure 1 shows a spark plug, partly in section and embodying certain features of my invention. Figs. 2 and 3 are diagrammatic sectional views of powder-testing means showing different angles of repose of powder.

In Fig. 1 there is shown the usual spark plug ceramic core 10 having a shoulder 11 seated upon a gasket 12 on the shoulder 13 of the usual shell 14. Above shoulder 11 the core is shown as being substantially cylindrical, and the bore of the shell is substantially cylindrical from shoulder 13 to an upper inturned flange 15. Beneath flange 15 there is a sealing ring 16. Beneath ring 16 and above shoulder 11 the space between the core and the shell is filled with compacted powder 17, which will be more fully described later.

The central electrode 18 is provided with a shoulder 19 which rests upon a shoulder 20 in the central bore of the core. Compacted powder 21 within the bore around the electrode and above the shoulder 19 seals the electrode in place, in a manner similar to that disclosed in my aforesaid co-pending application.

The powder I use for sealing the electrode in the core and the core in the shell must be readily

fed into the space to be filled and must be compatible by a permissible amount of pressure into a sealing body holding the parts in their respective positions and forming gas-tight joints and seals. As indicated in the aforesaid co-pending case, powdered soapstone is a material having these qualities. 5

I have discovered that other powdered mineral materials may be used that contain combined water but are dry so far as free water is concerned, and that do not lose water when heated to the temperature to which the several joints of the plug are subjected in regular use. Many materials have been tested and there are so few, if any, materials within the above definition 15 that cannot be compacted into an operative seal that the above definition appears to be a statement of the operative material sufficiently accurate for practical purposes.

The difficulty with powders of the kind described is that, even when rendered bone dry, so far as free water is concerned, by ordinary methods, the powder still has an undesirably high angle of repose. Of course any appreciable amount of free water in such powder interferes with its 25 pouring. For my purposes, a relatively low angle of repose is very advantageous.

Not only does a low angle of repose greatly facilitate the feeding of the powder into the space in which it is to be compacted, but it aids 30 in the uniform filling of such a space and lessens the danger of "bridging" during compacting. Where the powder has a high angle of repose, the attempt to compact any great depth in a narrow space is apt to result in "bridging", that 35 is, the compacting of an upper portion of the powder and its pressure against the adjacent walls sufficiently so that it is supported by friction on the walls and does not transmit pressure to the powder therebeneath. Under such 40 circumstances only the upper part of the powder is thoroughly compacted. Accordingly only a relatively shallow layer can be compacted at one time when the powder has a high angle of repose.

When the powder has a relatively low angle of repose, it acts more like a liquid during the initial stages of compression, and so is formed into a relatively uniform body before the final compression is applied. As a consequence, a deeper 50 layer in proportion to its width can be compressed at one operation.

In Fig. 2 there is shown a section of a box 25 having therein powder 26. One end 27 of the box is shown open, and, as indicated, the pow-

der runs out to a plane indicated at 28. This illustrates approximately the result with ordinary perfectly dry powdered soapstone where the angle of repose is above 50°, frequently about 55°. 5 Usually when the angle is 50° or over, the surface 28 is not smooth, but has irregularities therein, and when the box is tilted slightly, instead of flowing down evenly all over the surface, masses side here and there, in a manner aptly 10 described as "avalanching". It will be readily appreciated that powder in this condition is difficult to pack in a narrow space in a uniform manner.

However, soapstone powder or the like may be 15 treated, as by spray drying, so that it has an angle of repose of under 45°. In Fig. 3 there is illustrated a box 30 having therein powder 31, with one end 32 of the box open. Powder 31 has been treated so that it has an angle of repose 20 less than 45°, and, as illustrated, where the angle is less than 45° the surface 33 of the powder closely approximates a true plane, and tilting of the box results in a much more even flow of the material until the surface is restored to the 25 proper angle, with much less tendency to avalanche than when the angle of repose is higher.

It will be readily seen that such powder may be much more uniformly filled into a narrow space to considerable depth than where the angle 30 of repose is higher.

For satisfactory work in sealing electrodes into cores, I prefer to prepare the powder so that it has an angle of repose somewhat less than 45°. I have used with much success powdered soapstone treated and spray-dried so that it had an angle of repose of the order of 30°. While continued reduction of the angle of repose below 45° is helpful, it does not have as important an effect upon the behavior of the powder as does 40 the more critical change in the angle of repose from above 50° to below 45°.

Powder of the kind described may be readily 45 filled into the narrow space around the electrode, as well as between the core and shell, and may be compressed in a body which forms a gas-tight joint and frictionally engages the adjacent walls sufficiently to hold the assembled parts in place, and the compacted body has sufficient resiliency to maintain a tight joint between the parts throughout the repeated temperature changes to which the plug is subjected in use, and without imposing undue stresses upon the parts because of different coefficients of heat 55 expansion.

It is undesirable to permit access of moisture to the compacted powder, and therefore it is desirable to provide a substantially water-proof seal above the compacted powder. This may be done in various obvious ways.

A particularly desirable method of sealing the space above the powder between the core and shell is shown in Fig. 1, where the seal is made by ring 16 held in place by flange 15, but it 65 should be understood that the ring and flange are employed only for sealing the top of the space against the entrance of water or other injurious material, since the compacted powder securely holds the core and shell in assembled relation 70 with a constantly gas-tight joint, the powder gripping the shell and core sufficiently for this purpose. Obviously, other means may be substituted for protecting the joint from water, and other obvious changes may be made within the 75 scope of the appended claims.

What I claim is:—

1. The method of securing a ceramic spark plug core in a metallic shell which comprises assembling the core and shell in concentric relation with an annular space therebetween, filling said space with compactible powder, and compacting the powder until it forms a uniting body gripping the opposing walls of the parts and forming a gas-tight seal therebetween.

2. The method of securing together a conductor and a ceramic insulator, which comprises assembling the conductor and insulator in concentric relation with a narrow annular space therebetween, pouring into said space a non-metallic mineral powder, dry as to free water, containing 10 water of combination, and having an angle of repose of not over 45°, and compressing the powder in the space with sufficient force to compact it into a permanent holding body forming a gas tight joint with the opposed surfaces of the insulator and conductor, the filling and compressing being in successive layers which are sufficiently shallow to result in substantially uniform compacting of the powder without bridging.

3. The method of securing an electrode in a 20 rigid spark plug core, which consists in assembling the core and electrode with a space between the electrode and the surrounding wall of the bore of the core, pouring into said space a non-metallic mineral powder, dry as to free 30 water, containing water of combination that is not driven off at the temperature to which it is subjected in the use of the plug, and having an angle of repose of not over 45°, and compressing the powder in the space with sufficient force to 35 compact it into a permanent holding body forming a gas tight joint with the opposed surfaces of the insulator and conductor, the filling and compressing being in successive layers which are sufficiently shallow to result in substantially uniform 40 compacting of the powder without bridging.

4. The method of securing a rigid spark plug core in a metallic shell, which consists in placing the core in the shell with a space between their concentric surfaces, pouring into said space a 45 non-metallic mineral powder, dry as to free water, containing water of combination, and having an angle of repose of not over 45°, and compacting the powder in the space into a permanent holding body forming a gas-tight joint with said 50 concentric surfaces.

5. The method of securing a rigid spark plug core in a metallic shell, which consists in assembling the core and shell with a shoulder of the core resting on a shoulder of the shell and an 55 annular space between the core and shell above said shoulders, pouring into said space a non-metallic mineral powder, dry as to free water, containing water of combination, and having an angle of repose of not over 45°, and compacting 60 the powder in the space into a permanent holding body forming a gas-tight joint with the core and shell, and forming a water-tight seal above the compacted powder.

6. The method of securing a rigid spark plug core in a metallic shell, which consists in assembling the core and shell with a shoulder of the core resting on a shoulder of the shell and an annular space between the core and shell above said shoulders, pouring into said space a non- 70 metallic mineral powder, dry as to free water, containing water of combination, and having an angle of repose of not over 45°, and compacting the powder in the space into a permanent holding body forming a gas-tight joint with the core 75

and shell, fitting a ring above the compacted powder in substantially water-tight contact with the shell and core, and turning over the upper edge of the shell and thereby forming a flange holding the ring in place.

7. A spark plug comprising an electrode, a ceramic insulating core about the electrode, a metallic shell about said core, a seal between the electrode and core and between the core and shell, said seals consisting of powder compacted

in place and forming sealing and holding bodies. 8. A spark plug comprising a ceramic insulating core, a metallic shell around the core and providing a substantially cylindrical space inside the shell around the core, and powder compacted in said space into a holding and sealing body.

9. A spark plug in accordance with claim 8 and having a water-tight protection seal at the outer end of the compacted powder.

OTTO C. ROHDE. 10